

# United States Patent Office

3,083,162

Patented Mar. 26, 1963

1

3,083,162

## LUBRICATING COMPOSITION

Franklin I. L. Lawrence, Bradford, Pa., assignor to Kendall Refining Company, Bradford, Pa., a corporation of Pennsylvania

No Drawing. Filed Feb. 24, 1960, Ser. No. 10,559

13 Claims. (Cl. 252—33.4)

This invention relates to lubricating compositions and, more particularly, to lubricating compositions adapted to be added to gasoline fuels containing organolead, anti-knock compounds prior to the injection of the fuel into the combustion zone of an internal combustion engine.

In an effort to achieve maximum efficiency in gasoline internal combustion engines, a large number of additives have been proposed to reduce the deposits which occur within the combustion zone. Included in this wide variety of additives are alkaline earth metal sulfonates having an excess of metal (commonly termed "overbased" sulfonates) and chlorinated hydrocarbons.

Alkaline earth metal sulfonates are added to base oils and the like to provide improved detergent properties. With the use of such highly basic materials, sludging, carbon formation and ring sticking are reduced. Certain additives of this class, however, contribute to the formation of undesirable combustion chamber deposits, thereby inducing spark plug fouling.

Additionally, it is known that chlorinated hydrocarbons function as lead scavengers when incorporated into lead-containing gasoline fuels. The chlorine of the chlorinated hydrocarbons reacts with the lead during combustion to produce volatile lead compounds which pass from the combustion chamber. During combustion, non-volatile lead compounds tend to form which become deposited on the internal surfaces of the engine and thereby adversely affect the operation of the engine.

While the art has succeeded in extending engine life and in improving engine efficiency, the quest for even more effective additives or combination of additives continues.

Therefore, it is a primary object of the present invention to provide a lubricating composition which provides extended engine life.

It is an additional object of this invention to provide a lubricating composition adapted to be added to gasoline fuels prior to the injection of the fuel into an internal combustion engine.

It is another object of the present invention to provide a lubricating composition which promotes improved overall engine performance.

It is still another object of the present invention to provide a lubricating composition having excellent detergent properties.

It is a further object of the present invention to provide a lubricating composition which promotes improved spark plug performance.

Broadly stated, the present invention embraces a lubricating composition comprising a major amount of lubricating oil and (a) about 2.5 to about 3.5 weight percent of an oil-soluble alkaline earth metal sulfonate having a metal ratio of at least 2.25 selected from the group consisting of calcium, barium and strontium sulfonates and (b) an amount of a chlorinated hydrocarbon sufficient to provide between about 0.01 and about 0.015 equivalent of chlorine per 100 weight parts of lubricating composition.

The invention further contemplates a gasoline fuel containing the above defined lubricating composition.

While overbased sulfonates and chlorinated hydrocarbons are known additives, the conjoint utilization of these materials within the above defined critical limits has been found to produce a synergistic result. When, for example, either more chlorinated additive or less chlorinated

2

additive is employed, engine performance approximates that obtained employing other standard additives. When, however, the additives are employed within the critical ranges, engine performance is increased materially.

5 The alkaline earth metal sulfonates of the present invention embrace the oil-soluble alkaline earth metal salts of oil-soluble sulfonic acids which contain substantially more metal than is equivalent to the anionic radicals of the normal oil-soluble salts. The sulfonates generally 10 useful in the invention are disclosed, inter alia, in Patents Nos. 2,616,904, 2,616,905, 2,616,906, 2,616,910, 2,616,911, 2,616,924, 2,616,925, 2,617,049 and 2,723,235 to Asseff et al. The metal sulfonates employed in this invention have a metal ratio of at least about 2.25. Sulfonates may be characterized by a metal ratio up to 4.5 and higher.

15 As employed herein, the term "metal ratio" defines the ratio of equivalents of alkaline earth metal present in the sulfonate to equivalents of sulfonic acid groups. It will be apparent that the metal ratio of a neutral alkaline earth sulfonate is 1, and the metal ratio of a normal basic sulfonate (i.e.: R—SO<sub>3</sub>—Ca—OH) is 2.

20 The metals which form the sulfonates useful in the present invention are the alkali earth metals, strontium, barium and calcium. Calcium sulfonates are preferred for this invention.

25 The overbased sulfonates may be derived from sulfonic acids such as mahogany sulfonic acids; petrolatum sulfonic acids; mono- and polywax substituted naphthalene sulfonic, phenol sulfonic, diphenyl ether sulfonic, diphenyl ether disulfonic, naphthalene disulfide sulfonic, naphthalene disulfide disulfonic, diphenyl amine disulfonic, diphenyl amine sulfonic, thiophene sulfonic, alpha-chloro-naphthalene sulfonic acids, etc.; other substituted sulfonic acids such as cetyl chlorobenzene sulfonic acids, cetyl-phenol sulfonic acids, cetyl-phenol disulfide sulfonic acids, cetyl-phenol mono-sulfide sulfonic acids, cetoxy caprylbenzene sulfonic acids, di-cetyl thianthrene sulfonic acids, di-lauryl beta-naphthol sulfonic acids, and di-capryl nitro-naphthalene sulfonic acids; aliphatic sulfonic acids such as paraffin wax sulfonic acids, unsaturated paraffin wax sulfonic acids, hydroxy substituted paraffin wax sulfonic acids, tetraisobutylene sulfonic acids, tetraamylene sulfonic acids, chlorosubstituted paraffin wax sulfonic acids, nitroso paraffin wax sulfonic acids, etc.; cycloaliphatic sulfonic acids, such as petroleum naphthene sulfonic acids, bis-(diisobutyl)-cyclohexyl sulfonic acids, mono- and poly-wax substituted cyclohexyl sulfonic acids, etc.

30 35 40 45 50 55 60 Preparation of the alkaline earth metal sulfonates of the present invention may be carried out by any of the methods known to the art. For example, the overbased salts may be prepared by combining an inorganic alkaline earth compound with an oil-soluble sulfonic acid and/or the alkaline earth salt of the oil-soluble acid in the presence of a promoter, such as phenol. Such a method is exemplified inter alia in Asseff Patent No. 2,617,049. In such a manner, overbased sulfonates may be prepared which exhibit metal ratios up to about 4.5.

65 70 Additional information concerning the preparation of organic metal complexes suitable for the present invention can be found in the patents listed above.

The chloro hydrocarbons contemplated for use in the present invention include mono- and poly-chlorinated hydrocarbons which have a vapor pressure in the range of about 0.2 to about 6.0 mm. Hg at 50° C. These halogenated hydrocarbons include such chlorinated hydrocarbons as 1-chloronaphthalene, 1,8-dichlorooctane, dichloroxylanes (mixed), 3,4-dichlorocumene, pentachlorobutanes (mixed), hexachloropropylene, 1,2,4-trichlorobenzene, dichloroheptanes (mixed), 2,4-dichlorotoluene, 1,2-dichlorocyclohexane and 1-chlorooctane.

Preferred chlorinated hydrocarbons for utilization in the present invention constitute chlorinated benzene and mono- and poly-alkylated benzenes having from one to three carbon atoms in the alkyl chain and containing the chlorine attached to the benzene ring. Such compounds include, without limitation, chlorobenzenes, dichloroxylenes, monochloroxylenes, dichlorotoluenes, monochlorotoluenes, dichlorocumenes, monochlorocumenes, dichloroethylbenzenes, monochloroethylbenzenes, and the like. Dichlorotoluenes constitute a particularly preferred material for the practice of this invention.

The lubricating oil base useful in the present invention may be selected from any of the oils which find utility in lubricating compositions. They may be of vegetable, animal or mineral origin, but mineral oils, i.e., oils derived from petroleum, are preferred for the present invention. The properties of the base oil will depend upon the particular use and environment for which the lubricating composition is desired.

The lubricating compositions of this invention contain from about 2.5 to about 3.5 weight percent and preferably from about 2.8 to about 3.2 weight percent of oil-soluble alkaline earth metal sulfonates and sufficient chlorinated hydrocarbon to provide from about 0.01 to about 0.015 equivalent of chlorine and preferably from about 0.012 to 0.013 equivalent of chlorine per 100 weight units of lubricating composition.

It will be apparent that the base oil may contain other additives to improve such properties as the oiliness, pour point, and cold test without departing from the scope or spirit of the invention.

The components of the invention may be mixed by any method known to the art and in any sequence. The invention is not intended to be limited by the method of mixing the additive and the base oil.

The lubricating compositions of the present invention are ideally suited for use in engines wherein the lubricant is added with the gasoline fuel, such as, for example, two-cycle gasoline engines. Outboard motors, power saws, power mowers and the like constitute typical examples of equipment which may employ a two-cycle gasoline engine.

The lubricating compositions of this invention most appropriately may be employed in conjunction with gasoline fuels containing organolead anti-knock additives, such as tetraethyl lead, tetramethyl lead and the like. The gasoline fuels useful with the lubricating composition of this invention may be any of the leaded fuels of the gasoline range which find utility as fuels for internal combustion engines. Leaded gasolines are well-known to the art and, generally, contain from about  $\frac{1}{2}$  to about 4 or 5 cc. of tetraethyl lead per gallon of gasoline.

The lubricating composition of this invention may be employed in any desired amount in the gasoline. Normally, the lubricating compositions will be employed in amounts from about  $\frac{1}{4}$  to about 1 pint per gallon of gasoline, and preferably from about  $\frac{1}{3}$  to about  $\frac{2}{3}$  pints per gallon of gasoline. Blending may be effected in any desired manner.

The following specific embodiments are included for illustrative purposes only and in no way are intended to limit the scope of the invention.

#### EXAMPLE I

##### Test Procedure

The following procedure was employed to evaluate the high temperature-high speed performance characteristics of lubricating compositions:

A four-cylinder, 40-brake horsepower gasoline engine (Mercury Mark 55) was operated at a speed of  $5250 \pm 50$  r.p.m., with a jacket outlet temperature maintained at  $110-115^\circ$  F. The engine was operated at full throttle with a "load disk" instead of a propeller. The load disk was designed to absorb the rated load of approximately 40 b.h.p. at the 5250 r.p.m. of the engine.

The fuel employed in the tests was a mixture of 40% thermally cracked and 60% catalytically reformed gasoline containing 2.95 ml. tetraethyl lead, and characterized by the following properties:

|   |                        |        |        |
|---|------------------------|--------|--------|
| 5 | Gravity                | ° API  | 57.4   |
|   | Reid vapor pressure    | pounds | 9.8    |
|   | Distillation range     | ° F    | 97-403 |
|   | Research octane number |        | 93.3   |

10 The oil-to-gasoline ratio was maintained at 1 pint to 2 gallons.

The engine was operated until a spark plug fouled, as evidenced by a decrease of about at least 300 r.p.m. in the speed of the engine or an intermittent misfiring of the engine. All spark plugs then were changed. The test was terminated when three spark plugs had fouled.

The engine was disassembled and rated at the end of the test. Piston and port deposits and ring sticking were evaluated. The more important factors were 15 weighted in a summation of merit ratings. A "weighted total merit rating" of 100 denoted a perfectly clean engine.

Since the total test time varied because of variations in spark plug life, an overall measure of performance was 20 employed which accounted both for engine cleanliness and for the test time. "Weighted total merits" were multiplied by total test time to provide a "merit-hour rating." The "merit-hour rating" reflects good spark plug performance (long test in hours), as well as the ability of the oil 25 to keep the engine clean.

##### Lubricating Composition of This Invention

A lubricating composition was formulated which contained 3 weight percent of an overbased calcium sulfonate, 35 1% dichlorotoluene and 96% base oil.

The overbased calcium sulfonate analyzed 3.48% calcium, 2.34% sulfur and was characterized by a specific gravity of 1.00. The metal ratio of the calcium sulfonate was about 2.38.

40 The dichlorotoluene was characterized as follows:

|                  |                        |
|------------------|------------------------|
| $N_D^{20}$       | 1.5610                 |
| $d^{20}$         | 1.3952                 |
| Molecular weight | 198                    |
| Boiling range    | 185-209° C./730 mm. Hg |

45 51-53% chlorine

The amount employed provided a chlorine content of about 0.0125 equivalent of chlorine per 100 weight parts of lubricating composition.

50 Finally, the base oil employed was a heavy neutral, 90% raffinate produced as an overhead distillate from Pennsylvania base crude oil. The distillate was propane dewaxed and phenol extracted to a 90% raffinate yield. The oil was characterized by the following properties:

|                           |      |
|---------------------------|------|
| Viscosity at 100° F., SUS | 456  |
| Viscosity at 210° F., SUS | 61.7 |
| Viscosity index           | 99.8 |
| Pour point, ° F           | +10  |
| 55 Flash point, ° F       | 480  |
| Fire point, ° F           | 545  |
| Carbon residue, percent   | 0.19 |
| Gravity, ° API            | 29.3 |

60 The performance of the engine utilizing gasoline containing this additive is tabulated in Table 1 below.

|    |                       |        |
|----|-----------------------|--------|
| 65 | Weighted total merits | 77.87  |
|    | Total time            | 182:00 |
|    | Merit-hours           | 14,063 |
|    | Test time on plugs:   |        |
|    | 1st set               | 101:20 |
|    | 2nd set               | 44:15  |
| 70 | 3rd set               | 36:25  |

**5**  
**EXAMPLE II**

In order to demonstrate the effect of the overbased calcium sulfonate employed as a sole additive to the lubricating oil, two tests were conducted employing 2 weight percent of the overbased calcium sulfonate described in Example I above. In all other respects, the tests were identical with those described in Example I above.

The results of these tests are reflected in Table 2 below.

TABLE 2

|                                       | Test No. |       |
|---------------------------------------|----------|-------|
|                                       | 2        | 3     |
| Compounding data:                     |          |       |
| Base oil                              | 98.0     | 98.0  |
| Additive, overbased calcium sulfonate | 2.0      | 2.0   |
| Weighted total merits                 | 81.51    | 85.00 |
| Total time                            | 63:20    | 37:20 |
| Merit-hours                           | 5,162    | 3,173 |
| Test time on plugs:                   |          |       |
| 1st set                               | 26:20    | 33:20 |
| 2nd set                               | 15:10    | 3:10  |
| 3rd set                               | 21:50    | 0:50  |

## EXAMPLE III

In order to demonstrate the effect of the dichlorotoluene employed alone, 2 weight percent of the dichlorotoluene were admixed with the base oil of Example I. The results of the test wherein the lubricating composition contained approximately 0.025 equivalent of chlorine per 100 weight parts of lubricating composition are reflected in Table 3 below.

TABLE 3

|                           |            |
|---------------------------|------------|
| Compounding data:         | Test No. 4 |
| Base oil                  | 98.0       |
| Additive, dichlorotoluene | 2.0        |
| Weighted total merits     | 68.46      |
| Total time                | 80:00      |
| Merit-hours               | 5477       |
| Test time on plugs:       |            |
| 1st set                   | 51:35      |
| 2nd set                   | 15:40      |
| 3rd set                   | 12:45      |

## EXAMPLE IV

In order to demonstrate the optimum range of overbased sulfonate and chlorinated hydrocarbon, tests similar to Example I were conducted employing the same lubricating composition ingredients, but varying amounts of dichlorotoluene. The data from these tests is reflected in Table 4 below. In test No. 5 the chlorine content of the lubricating composition was about 0.00625 equivalent per 100 weight units of lubricating composition and the chlorine content in test No. 6 was about 0.025 equivalent of chlorine per 100 weight units of the lubricating composition.

TABLE 4

|                             | Test No. |         |
|-----------------------------|----------|---------|
|                             | 5        | 6       |
| Compounding data:           |          |         |
| Base oil                    | 96.5     | 95.0    |
| Additive:                   |          |         |
| Overbased calcium sulfonate | 3.0      | 3.0     |
| Dichlorotoluene             | 0.5      | 2.0     |
| Weighted total merits       | 88.28    | 80.00   |
| Total time                  | 72:20    | 1 48:45 |
| Merit-hours                 | 6024     |         |
| Test time on plugs:         |          |         |
| 1st set                     | 60:35    | 1 48:45 |
| 2nd set                     | 9:05     |         |
| 3rd set                     | 2:40     |         |

<sup>1</sup> Terminated at drive train gear failure.

While drive train gear failure terminated test No. 6 at the end of 48 hours, the "weighted total merits" of that

test make it apparent that the lubricating composition therein employed was substantially less efficient than that exemplified in Example III above.

5

**6**

In order to demonstrate further the effectiveness of the lubricating compositions of this invention, two commercial outboard motor oils were employed in the test procedure described in Example I. Oil A was a 100% naphthenic distillate and contained no apparent additives and was characterized by the following properties:

|                           |      |
|---------------------------|------|
| Viscosity at 210° F., SUS | 59.6 |
| Viscosity at 100° F., SUS | 763  |
| Viscosity index           | 1.0  |
| Pour point, ° F           | +5   |
| Flash point, ° F          | 420  |
| Fire point, ° F           | 465  |

Oil B was a solvent refined oil containing overbased barium sulfonate and zinc dithiophosphate additives. Its properties were characterized as follows:

|                           |       |
|---------------------------|-------|
| Viscosity at 210° F., SUS | 62.6  |
| Viscosity at 100° F., SUS | 476   |
| Viscosity index           | 99    |
| Pour point, ° F           | -25   |
| Flash point, ° F          | 445   |
| Fire point, ° F           | 495   |
| Sulfur, percent           | 0.55  |
| Phosphorous, percent      | 0.03  |
| Barium, percent           | 0.125 |
| Zinc, percent             | 0.04  |

The results of the tests conducted employing oils A and B are reflected in Table 5 below. The data from test No. 8 particularly reflect the tendency of certain detergent additives with appreciable metal content to promote spark plug fouling.

40

TABLE 5

|                       | Test No. |          |
|-----------------------|----------|----------|
|                       | 7, oil A | 8, oil B |
| Weighted total merits | 78.13    | 72.04    |
| Total time            | 34:25    | 20:00    |
| Merit-hours           | 2,689    | 1,441    |
| Test time on plugs:   |          |          |
| 1st set               | 22:40    | 7:10     |
| 2nd set               | 11:45    | 10:20    |
| 3rd set               | 0:00     | 2:30     |

## EXAMPLE VI

Still further to demonstrate the effectiveness of the additive of this invention, tests were conducted employing the base oil identified in Example I, free of additives.

The results of these tests are reflected in Table 6 below.

60

TABLE 6

|                       | Test No. |       |       |       |
|-----------------------|----------|-------|-------|-------|
|                       | 9        | 10    | 11    | 12    |
| Compounding data:     |          |       |       |       |
| Base oil              | 100.0    | 100.0 | 100.0 | 100.0 |
| Weighted total merits | 67.70    | 74.95 | 74.89 | 77.50 |
| Total time            | 44:15    | 32:40 | 32:10 | 31:35 |
| Merit-hours           | 2,996    | 2,449 | 2,409 | 2,447 |
| Test time on plugs:   |          |       |       |       |
| 1st set               | 29:15    | 32:30 | 25:45 | 23:00 |
| 2nd set               | 14:30    | 0:10  | 4:25  | 3:55  |
| 3rd set               |          |       | 2:00  | 4:40  |

## EXAMPLE VII

Additional additives were tested to determine their

efficiency in the tests described in Example I. The results of these tests are reflected in Table 7 below.

TABLE 7

|                       | Test No. |       |       |       |       |       |       |       |
|-----------------------|----------|-------|-------|-------|-------|-------|-------|-------|
|                       | 13       | 14    | 15    | 16    | 17    | 18    | 19    | 20    |
| Compounding data:     |          |       |       |       |       |       |       |       |
| Base oil.....         | 99.44    | 98.5  | 98.4  | 99.5  | 98.8  | 99.5  | 99.2  | 97.0  |
| Additive:             |          |       |       |       |       |       |       |       |
| A.....                |          | 1.5   |       |       |       |       |       |       |
| B.....                |          |       | 1.6   |       |       | 1.2   |       |       |
| C.....                |          |       |       |       | 0.5   |       |       |       |
| D.....                |          |       |       |       |       |       |       |       |
| E.....                | 0.56     |       |       |       |       | 0.5   |       |       |
| F.....                |          |       |       |       |       |       | 0.8   |       |
| G.....                |          |       |       |       |       |       |       | 0.2   |
| Weighted total merits | 78.25    | 91.00 | 84.60 | 86.84 | 66.69 | 73.47 | 66.30 | 91.29 |
| Total time.....       | 32:45    | 25:45 | 36:00 | 11:20 | 54:20 | 49:30 | 26:15 | 31:35 |
| Merit-hours.....      | 2,563    | 2,343 | 2,961 | 984   | 3,023 | 8,537 | 1,740 | 2,883 |
| Test time on plugs:   |          |       |       |       |       |       |       |       |
| 1st set.....          | 24:45    | 21:30 | 25:30 | 5:08  | 30:50 | 28:30 | 18:00 | 23:00 |
| 2nd set.....          | 7:50     | 3:50  | 4:50  | 2:10  | 17:20 | 12:00 | 8:00  | 5:50  |
| 3rd set.....          | :10      | 0:25  | 4:40  | 4:05  | 6:10  | 9:00  | 0:05  | 2:45  |

The above lettered additives are identified as follows:

| Additive | Chemical composition                                                                                                   | Properties                                             |
|----------|------------------------------------------------------------------------------------------------------------------------|--------------------------------------------------------|
| A.....   | Low molecular weight polymethacrylate containing nitrogen functional groups plus a phosphorous extreme pressure agent. | 5.3% nitrogen, 1.7% phosphorous.                       |
| B.....   | Lead alkyl phenate.....                                                                                                | 16.5% lead, specific gravity 1.10.                     |
| C.....   | P <sub>2</sub> S <sub>5</sub> , terpene reaction product.....                                                          | 4.7% phosphorous, 13.0% sulfur, 1.02 specific gravity. |
| D.....   | Bis-B-chloroethyl vinyl phosphonate.....                                                                               | 29.8% chlorine, 13.3% phosphorous.                     |
| E.....   | Tricresyl phosphate.....                                                                                               | 8.4% phosphorous, molecular weight 368.                |
| F.....   | 4,4-methylenbis (2,6-di-tert-butyl phenol).                                                                            |                                                        |
| G.....   | Sorbitol monooleate.....                                                                                               | Specific gravity 1.00.                                 |

It will be apparent that the gasolines to which the additives of this invention have been added may contain other standard additives well-known to the art.

Since modifications of the present invention will be apparent to those skilled in the art, the invention is intended to be limited only by the scope of the appended claims.

I claim:

1. A lubricating composition comprising a major amount of lubricating oil and (a) from about 2.5 to about 3.5 weight percent of an oil-soluble alkaline earth metal sulfonate having a metal to sulfonic acid group equivalent ratio of at least 2.25 selected from the group consisting of calcium, barium, and strontium sulfonates and (b) an amount of a chlorinated hydrocarbon selected from the group consisting of mono- and poly-chlorinated hydrocarbons having a vapor pressure in the range of about 0.2 to about 6.0 mm. of mercury at 50° C. sufficient to provide between about 0.01 and about 0.015 equivalent of chlorine per 100 weight parts of lubricating composition.

2. The lubricating composition of claim 1 wherein the metal sulfonate is present in amounts from about 2.8 to about 3.2 weight percent.

3. The lubricating composition of claim 1 wherein the chlorinated hydrocarbon is present in amounts sufficient to provide between about 0.012 and 0.013 equivalent of chlorine per 100 weight units of lubricating composition.

4. The lubricating composition of claim 1 wherein the

sulfonate is present in amounts from about 2.8 to about 3.2 weight percent and the chlorinated hydrocarbon is present in amounts sufficient to provide between about 0.012 and 0.013 equivalent of chlorine per 100 weight units of lubricating composition.

5. The lubricating composition of claim 1 wherein the chlorinated hydrocarbon is selected from the group consisting of chlorinated benzene and mono- and poly-alkylated benzenes having from 1 to 3 carbon atoms in the alkyl chain and containing the chlorine attached to the benzene ring.

6. The lubricating composition of claim 1 wherein the alkaline earth metal sulfonate is a calcium sulfonate.

7. A lubricating composition comprising a major amount of lubricating oil and (a) from about 2.5 to about 3.5 weight percent of an oil-soluble calcium sulfonate having a metal to sulfonic acid group equivalent ratio of about 2.38 and (b) dichlorotoluene in an amount sufficient to provide between about 0.01 and about 0.015 equivalent of chlorine per 100 weight parts of lubricating composition.

8. A leaded gasoline containing a lubricating amount of a lubricating composition comprising a major amount of lubricating oil and (a) from about 2.5 to about 3.5 weight percent of an oil-soluble alkaline earth metal sulfonate having a metal to sulfonic acid group equivalent ratio of at least 2.25 selected from the group consisting of calcium, barium, and strontium sulfonates and (b) an amount of a chlorinated hydrocarbon selected from the group consisting of mono- and poly-chlorinated hydrocarbons having a vapor pressure in the range of about 0.2 to about 6.0 mm. of mercury at 50° C. sufficient to provide between about 0.01 and about 0.015 equivalent of chlorine per 100 weight parts of lubricating composition.

9. The leaded gasoline of claim 8 containing from about 1/4 to about 1 pint of lubricating composition per gallon of gasoline.

10. The leaded gasoline of claim 8 containing from about 1/2 to about 2/3 pint of lubricating composition per gallon of gasoline.

11. A leaded gasoline containing a lubricating amount of a lubricating composition comprising a major amount of lubricating oil and (a) from about 2.5 to about 3.5 weight percent of an oil-soluble calcium sulfonate having a metal to sulfonic acid group equivalent ratio of about 2.38 and (b) dichlorotoluene in an amount sufficient to provide between about 0.01 and about 0.015 equivalent of chlorine per 100 weight parts of lubricating composition.

12. The leaded gasoline of claim 11 containing from about 1/4 to about 1 pint of lubricating composition per gallon of gasoline.

13. The leaded gasoline of claim 11 containing from about 1/2 to about 2/3 pint of lubricating composition per gallon of gasoline.

#### References Cited in the file of this patent

#### UNITED STATES PATENTS

|           |                   |               |
|-----------|-------------------|---------------|
| 2,968,635 | Prutton           | Jan. 19, 1937 |
| 2,364,921 | Shokal            | Dec. 12, 1944 |
| 2,479,903 | Calingaert et al. | Aug. 23, 1949 |
| 2,585,520 | Van Ess et al.    | Feb. 12, 1952 |
| 2,913,412 | Moore et al.      | Nov. 17, 1959 |
| 2,935,476 | Stuart            | May 3, 1960   |
| 2,950,960 | Barusch et al.    | Aug. 30, 1960 |